

# United States Patent [19]

Wilson

[11]

4,293,305

[45]

Oct. 6, 1981

[54] **DIESTER COMPOSITION AND TEXTILE PROCESSING COMPOSITIONS THEREFROM**

[75] Inventor: **Robert B. Wilson**, Greenville, S.C.

[73] Assignee: **Northwestern Laboratories, Inc.**, Greenville, S.C.

[21] Appl. No.: **203,636**

[22] Filed: **Nov. 3, 1980**

**Related U.S. Application Data**

[63] Continuation-in-part of Ser. No. 90,092, Nov. 1, 1979.

[51] Int. Cl.<sup>3</sup> ..... **D06M 1/00**

[52] U.S. Cl. ..... **8/115.6; 8/116 P;**  
8/922; 252/8.6; 252/8.9; 260/97.5; 428/265;  
428/395; 560/128

[58] **Field of Search** ..... **8/115.6, 116 P;**  
252/8.6, 8.9; 428/265, 395; 260/97.5; 560/128

[56] **References Cited**

**U.S. PATENT DOCUMENTS**

3,329,633 7/1967 Crovatt ..... 8/115.6  
3,694,257 9/1972 Dumont ..... 428/262  
3,753,968 8/1973 Ward ..... 260/97.5  
3,899,476 8/1975 Ward ..... 260/97.5  
3,925,589 12/1975 Sturwold et al. ..... 528/491  
3,950,419 4/1970 Baumann et al. ..... 8/115.6  
4,135,878 1/1979 Bishop et al. ..... 8/115.6

**OTHER PUBLICATIONS**

Ward, B. F. et al., J. Amer. Oil Chemists' Soc., 1975, 52, (No. 7), pp. 219-224.

Teeter, H. M. et al., J. Organic Chemistry, 1957, 22, 512-514.

Danzig, M. J. et al., J. Amer. Oil Chemists' Soc., 1957, 34, pp. 136-138.

Teeter, H. M. et al., J. Amer. Oil Chemists' Soc., 1938, 35, pp. 238-240.

*Primary Examiner*—A. Lionel Clingman  
*Attorney, Agent, or Firm*—Bailey, Dority & Flint

[57]

**ABSTRACT**

A cycloaliphatic diester of the formula



wherein

R is straight or branched chain alkyl of 4-20 carbon atoms, polyoxyalkylene of the formula  $\text{HO}(\text{CH}_2\text{C}_2\text{H}_2\text{O})_n\text{CH}_2\text{CH}_2-$ ,  $\text{HO}(\text{C}_3\text{H}_6\text{O})_n\text{C}_6\text{H}_3-$ ,  $\text{HO}(\text{CH}_2\text{C}_2\text{H}_2\text{O})_p(\text{C}_3\text{H}_6\text{O})_q\text{C}_3\text{H}_6-$ , or  $\text{HO}(\text{C}_3\text{H}_6\text{O})_p(\text{C}_2\text{H}_4\text{O})_q\text{C}_2\text{H}_4-$  or phosphated polyoxyalkylene, wherein n is 2-22 and the sum of p+q is n, in combination with a high boiling aromatic ester, is useful in fiber treating and textile processing compositions.

**5 Claims, 4 Drawing Figures**



**CONVENTIONAL SPIN FINISH  
(200X)**



**Fig. 1**  
CONVENTIONAL SPIN FINISH  
(200X)



**Fig. 2**  
FINISH OF EXAMPLE 15  
(200X)



**Fig. 3**  
CONVENTIONAL SPIN FINISH  
(400X)



**Fig. 4**  
FINISH OF EXAMPLE 15  
(400X)

## DIESTER COMPOSITION AND TEXTILE PROCESSING COMPOSITIONS THEREFROM

### REFERENCE TO RELATED APPLICATIONS

This is a continuation-in-part of Ser. No. 090,092, filed Nov. 1, 1979.

### BACKGROUND OF THE INVENTION

This invention relates to a combination of cycloaliphatic diesters and high boiling aromatic esters and their use in fiber-treating and textile processing compositions.

### PRIOR ART STATEMENT

It has been proposed by Sturwold et al, in U.S. Pat. No. 3,925,589, to use emulsions of esters derived from polyoxy-alkylene glycols of molecular weight 300-4000 and a dibasic acid mixture of a dimer acid of 32-54 carbon atoms and a short chain dibasic acid of 2-12 carbon atoms for lubricating polyamide fibers.

Dumont, in U.S. Pat. No. 3,694,257, has proposed the use of polyesters prepared from reaction of polyols with a di- or tribasic acid as textile assistants for softening textile fabrics.

It has been proposed by Crovatt, Jr., in U.S. Pat. No. 3,329,633, to improve the lubricity of polyhexamethylene adipamide fibers by adding 0.1-5.0% by weight of oleic acid dimer to the polymer during the final polymerization stage thereof.

Bishop et al, in U.S. Pat. No. 4,135,878, has disclosed inclusion of up to 10% by weight of a dimer acid in an emulsifier-solvent scour composition used for treating textile materials under alkaline conditions.

Preparations of adducts from conjugated octadecadienoic acid and unsaturated acids and/or their hydrogenation has been described by Teeter et al, J. Org. Chem., vol. 22 (1957) at 512-514, Ward in U.S. Pat. No. 3,899,476 and Ward et al in U.S. Pat. No. 3,981,682.

The preparation of esters from the C<sub>21</sub> diacid adduct was reported by Ward et al, J. Amer. Oil Chemists' Soc., vol. 57 (1975) at 219-224. Ethoxylated esters containing 4-119 ethylene oxide units are said to be particularly effective lime soap dispersants. The alkyl esters are reported as being particularly useful in lubricant applications, including uses as textile lubricants and plasticizers for PVC.

The use of lower aromatic esters in textile treatment, particularly as dyeing assistants is well known, as is disclosed in U.S. Pat. Nos.: 2,880,050 Fortress et al; 2,881,045 Mecco et al; 3,036,876 Schoellig et al; 3,124,412 Fidell et al; 3,929,407 Parker; 3,932,128 Beau lieu.

References which disclose the use of phthalate esters in dyeing processes include U.S. Pat. Nos.: 2,833,613 Hallada et al; 2,934,397 Landeri; 2,982,597 Salvin et al; 3,667,899 Harnett et al; 3,973,907 Forschirm; 4,032,291 Delilian.

Phthalate esters have been used as components of lubricants for textiles, for example, by Jaeger (U.S. Pat. No. 2,212,369), Dickey et al (U.S. Pat. No. 2,241,246), Brennan et al (U.S. Pat. No. 2,882,231) and Iyengar et al (U.S. Pat. No. 3,853,607).

The use of hydroxyalkyl or alkoxyalkyl benzoates as dyeing assistants or fixatives is disclosed by Fuhr et al (U.S. Pat. No. 3,532,454), Baumann et al (U.S. Pat. No. 3,950,419) and Lazar et al (U.S. Pat. No. 3,917,447).

Higher trialkyl trimellitates have been proposed by Hinton, Jr. et al as components of a soil release composition (U.S. Pat. No. 3,824,125).

### OBJECT OF THE INVENTION

It is an object of the invention to provide a novel combination of cycloaliphatic and high boiling aromatic esters which, used as ingredients of textile-processing agents, particularly for polyester fibers, eliminates one or more otherwise conventional processing steps without impairing the ultimate properties of the fiber treated therewith.

### SUMMARY OF THE INVENTION

In one aspect of this invention, cycloaliphatic diesters of the formula



wherein A is  $-\text{CH}_2-\text{CH}_2-$  and R is straight or branched chain alkyl of 4-20 carbon atoms, polyoxyalkylene of the formula  $\text{HO}(\text{C}_x\text{H}_y\text{O})_n\text{C}_x\text{H}_y-$  or phosphated polyoxyalkylene of the formula



or a salt thereof wherein  $(\text{C}_x\text{H}_y\text{O})_n$  is  $(\text{CH}_2\text{CH}_2\text{O})_n$ ,  $(\text{C}_3\text{H}_6\text{O})_n$  or  $(\text{CH}_2\text{CH}_2\text{O})_p(\text{C}_3\text{H}_6\text{O})_q$  and n is 2-22 are combined with a high boiling aromatic ester of the formula  $\text{ArCOO-R}_1\text{OCOAr}$  or  $\text{ArCOOR}_2$ , wherein Ar is monocyclic aryl of up to 10 carbon atoms; R<sub>1</sub> is alkylene of up to 8 carbon atoms, or polyoxyalkylene of the formula  $-\text{C}_x\text{H}_{2r}(\text{O}-\text{C}_x\text{H}_2)_s-$  in which r is 2 or 3 and s is up to 15; and R<sub>2</sub> is alkyl or alkenyl of 8-30 carbon atoms, to provide a base for a multi-purpose fiber and textile-treating composition.

This invention further relates to a synthetic fiber or fabric coated with a treating-agent containing the foregoing composition.

This invention further relates in the conversion of synthetic fibers to piece goods and subsequent dyeing, to the improvement wherein a composition of this invention is the sole fiber-treating agent used.

This invention also relates to a method of making fabric or an article from a synthetic fiber or fabric comprising coating the fiber or fabric with 1-2% by weight of a knitting or weaving lubricant comprising 5-15 parts by weight of cycloaliphatic diester, 30-50 parts by weight of high boiling aromatic ester, 5-15 parts by weight of dye-levelling agent and 10-30 parts by weight of emulsifiers, dispersing agents and/or anti-static agents; knitting or weaving the fiber into fabric or a knitted or woven article and dyeing the fabric or knit or woven article.

This invention further relates to a method for treating a synthetic fiber comprising applying to the fiber to a pick-up of 0.4-0.75% by weight a spin finish comprising (1) a cycloaliphatic diester, (2) a high boiling aromatic diester and (3) a dye-levelling agent; texturing the thus-coated synthetic fiber at 180°-230° C.; knitting or weaving the resulting textured fiber into fabric or knitting the

textured fiber into a knit article and dyeing the fabric or knit article.

In another aspect, this invention relates to a method for lowering heat history characteristics and the degree of crystallinity of a synthetic fiber, lowering the temperature at which the fiber can be texturized and lowering the temperature at which the fiber absorbs dye comprising applying to the fiber to a pick-up of 0.4-0.75% by weight of a composition comprising a cycloaliphatic diester and a high boiling aromatic ester, wherein the ratio of cycloaliphatic diester to high boiling aromatic ester is 0.1:1 to 2:1 and wherein the combination of cycloaliphatic diester and high boiling aromatic constitutes 10-90% by weight of the composition and texturing the thus-coated fiber at 180°-230° C. Moreover, aforesaid composition can contain a dye-leveling agent of the formula  $R_3COOR_4$ .

#### BRIEF DESCRIPTION OF THE DRAWING

In FIG. 1-4 are shown representations of photomicrographs of polyester yarn treated with the composition of Example 15 and with a conventional spin finish composition.

#### DETAILED DISCUSSION

The dibasic acid employed in making the compositions of this invention is a Diels-Alder adduct of acrylic acid and linoleic acid and can be prepared as described by Ward in U.S. Pat. No. 3,753,968. The diacid has the formula



and therefore is a mixture of (5 and 6)-carboxy-4-hexyl-2-cyclohexene-1-octanoic acids. The diacid is available commercially from Westvaco, designated as "Diacid 1500".

The diacid can be esterified with alcohols using, for example, acidic catalysts such as p-toluenesulfonic acid, methanesulfonic acid or sulfuric acid. During the esterification, the reaction mixture is preferably also treated with a decolorizing agent, e.g., carbon or clay.

The diacid is reduced following esterification to a compound in which A is  $-\text{CH}_2\text{CH}_2-$ . A nickel catalyst such as Raney Nickel, nickel on kieselguhr or nickel on alumina can be used. The required amount varies up to 5-10% by weight of the ester.

Hydrogenation is carried out after esterification to prevent nickel from complexing with the free acid. Other catalysts, e.g., platinum or rhodium, avoid this problem, but are prohibitive in cost. The catalyst can be removed by filtration through a plate and frame filter press. The product is the resulting filtrate.

Polyoxyalkylene diesters are prepared by reaction of the diacid, in the presence of an alkaline catalyst, with ethylene or propylene oxide. Reaction will occur at both acid sites and addition of ethylene oxide is allowed to continue until the product becomes at least dispersible or, preferably, soluble in water. This will correspond to addition of a total of 5-25 ethylene oxide units. The product obtained using ethylene oxide has a structure before hydrogenation represented by the formula:



The phosphorylated product is readily obtained by reaction with phosphorus pentoxide. The saturated diester can be obtained by nickel-catalyzed hydrogenation.

In the case of the phosphorylated derivative, hydrogenation should precede phosphorylation. The phosphorylated derivatives can be converted to salts thereof by reaction with a metal hydroxide. Sodium and potassium salts are preferred.

It will be understood that the diesters used in the compositions of this invention have somewhat varying properties. However, the following general correlation between structure and properties of representative preferred diesters (hydrogenated form) can be made:

|    |                                                               |                               |
|----|---------------------------------------------------------------|-------------------------------|
| 25 | dilauryl ester                                                | liquid, good heat stability,  |
|    | bis(2-ethylhexyl)ester                                        | liquid, good heat stability,  |
| 30 | distearyl ester                                               | good lubricant                |
|    | bis(ethoxylated)ester<br>(15 moles ethylene oxide)            | solid, good heat stability,   |
|    | bis(phosphated ethoxylated)ester<br>(15 moles ethylene oxide) | good lubricant                |
|    |                                                               | solid, heat stable, cohesive  |
|    |                                                               | solid, heat stable, cohesive, |
|    |                                                               | antistatic                    |

Preferred diesters for use in accordance with the principles of the invention are those wherein: A is  $-\text{CH}_2\text{CH}_2-$  and

- (a) R is straight or branched chain alkyl of 4-20 carbon atoms,
- (b) R is 2-ethylhexyl, lauryl or stearyl,
- (c) R is  $\text{HO}(\text{CH}_2\text{CH}_2\text{O})_n\text{CH}_2\text{CH}_2-$ ,
- (d) R is  $\text{HO}(\text{C}_3\text{H}_6\text{O})_n\text{C}_3\text{H}_6-$ ,
- (e) R is  $\text{HO}(\text{C}_2\text{H}_4\text{O})_p(\text{C}_3\text{H}_6\text{O})_q\text{C}_3\text{H}_6-$ , and



It will be understood that the textile-treating compositions can contain more than one diester, e.g., a mixture of bis(alkyl) esters or a mixture containing a bisalkyl ester in combination with a bis(polyoxyalkylene) or bis(phosphated polyoxyalkylene) ester of a corresponding salt.

"High boiling aromatic ester" as used in the specification and claims means an ester of the formula  $\text{ArCOO-R}_1-\text{OOCAr}$  or  $\text{ArCOOR}_2$ , wherein Ar is monocyclic aryl of up to 10 carbon atoms;  $R_1$  is alkylene of 2-8 carbon atoms or polyoxyalkylene of the formula  $-\text{C}_r\text{H}_{2r}(\text{O-C}_s\text{H}_{2s})_s$ , in which r is 2 or 3 and s is up to 15; and  $R_2$  is alkyl or alkenyl of 8-30 carbon atoms.

Accordingly, aromatic esters used in the practice of this invention include, but are not limited to, esters of benzoic, toluic, dimethylbenzoic, trimethylbenzoic, butylbenzoic and similar acids.

In the case of aromatic diesters, alkylene ( $R_1$ ) can be ethylene, propylene, hexylene, 2,2-dimethyl-trimethylene, butylene, heptamethylene and octylene, including various isomers thereof.

Polyoxyalkylene diesters include those derived from polyethylene glycol or polypropylene glycol.

In the case of monoaromatic esters, alkyl can be octyl, nonyl, decyl, dodecyl, tridecyl, hexadecyl, stearyl and alkenyl can be any corresponding monounsaturated function, e.g., oleyl.

Preferred aromatic diesters are those wherein:

- (a) Ar is phenyl,
- (b) Ar is tolyl,
- (c) R<sub>1</sub> is ethylene or propylene, including each of (a) and (b),
- (d) R<sub>1</sub> is ethyleneoxyethylene or propyleneoxypropylene, including each of (a) and (b),
- (e) R<sub>1</sub> is polyoxypropylene of molecular weight 200-500, including each of (a) and (b), and
- (f) R<sub>2</sub> is decyl, dodecyl, hexadecyl, tridecyl, octadecyl or oleyl, including each of (a) and (b).

It has been found that aromatic esters falling outside of the foregoing definition, more particularly methyl, ethyl, propyl, butyl, pentyl and hexyl benzoates, lack heat stability, low odor and lubricating properties required for the plurality of functions fulfilled by the compositions of this invention.

Ethoxylated castor oil used in the compositions will contain 15-100 oxyethylene units, preferably 40-85. The hydrogenated castor oil derivatives will contain 5-200 oxyethylene units, preferably 20-30. These materials can be purchased from ICI America and White-stone Chemical.

Ethoxylated alkyl phenols used in the compositions of this invention will contain up to 12 carbon atoms in the alkyl function and from 1-25 ethylene oxide units. Preferred examples are ethoxylated nonylphenol having 10-15 ethylene oxide units.

Ethoxylated alkanols include those derived from 12-15 carbon alkanols, including mixtures thereof, or from secondary alcohols of 11-15 carbon atoms, also including mixtures, and containing 6-15 ethylene oxide units.

Phosphated ethoxylated alkanols or phenols employed in the compositions of the invention will generally have fewer ethyleneoxide units than the unphosphated compounds. Exemplary, but not limitative, of the materials which can be used are the potassium salts of POE (10) nonylphenol phosphate, POE (3.5) lauryl alcohol phosphate, POE (7) lauryl alcohol phosphate, POE (9) lauryl alcohol phosphate, POE (6) decyl alcohol phosphate, and POE (9) decyl alcohol phosphate. It will be understood that the formula given for the phosphated ethoxylated derivatives includes various products, including phosphated mono- and diesters, obtained by reaction between the ethoxylated diacids and P<sub>2</sub>O<sub>5</sub>.

In many cases, the composition of this invention will be left on the fiber during dyeing and will therefore function as dyeing assistants in which case, 10-25% by weight of a dye-levelling agent will be included. "Dye-levelling agent," as used in the specification and claims, will be of the formula R<sub>3</sub>COOR<sub>4</sub>, wherein R<sub>4</sub> is an ethoxylated alkylphenol residue of the formula



a is 0-12 and b is 1-24 or an ethoxylated alkanol residue of the formula



c is 7-12 and d is 1-24 and wherein R<sub>3</sub> is linear or branched alkyl or alkenyl of 1-21 carbon atoms, phenyl or tolyl.

Accordingly, exemplary dye-levelling agents include laurate, myristate, palmitate, coconutate, oleate, stearate, isostearate, benzoate and toluate esters of ethoxylated nonylphenol, octylphenol, dodecylphenol, n-decanol, n-dodecanol, n-tetradecanol or n-hexadecanol. The extent of ethoxylation is from 1-25 ethylene oxide units per alkylphenol or alkanol, preferably 6-15 ethylene oxide units.

Preferred dye-levelling agents are those wherein:

- (a) R<sub>3</sub> is of 11-17 carbon atoms, including mixtures thereof;
- (b) R<sub>3</sub> is n-C<sub>17</sub>H<sub>33</sub>;
- (c) R<sub>3</sub> is n-C<sub>17</sub>H<sub>35</sub>;
- (d) R<sub>3</sub> is iso-C<sub>17</sub>H<sub>35</sub>;
- (e) R<sub>3</sub> is phenyl;
- (f) R<sub>3</sub> is n-C<sub>11</sub>H<sub>23</sub>;
- (g) a is 9, including each of (a)-(f);
- (h) c is 11-14, including mixtures thereof and including each of (a)-(f);
- (i) b is about 9.5, including each of (a)-(f);
- (j) d is 6-10, including each of (a)-(f);
- (k) b is 6-15, including each of (a)-(f); and
- (l) a is 9, b is 8-10 and R<sub>3</sub> is n-C<sub>11</sub>H<sub>23</sub>.

The compositions are especially suited for treatment of synthetic fibers such as polyester, polyamide, and polyacrylic. The polyester may be spun or textured polyester or filament or warp yarn and may be woven, knitted, tufted, needle punched or non-woven. The polyester can be a polyalkylene terephthalate, such as polyethylene terephthalate, or a polyester made from cyclohexane-dimethanol. The polyamide may be of types 6, 6,6 or 6,10. The acrylic may be straight acrylic (acrylonitrile) or modacrylic (modified with vinyl chloride, vinylidene chloride). The compositions are also adapted for application to blends of the above fibers with each other and with cellulosics (cotton, rayon, etc.) of wool.

The compositions can be applied at any of several stages of fiber processing. The following are exemplary of application to polyester fiber:

#### A. Spin Finish Application:

The composition is applied to the yarn from a 10-20% emulsion to give a finish level on the yarn of 0.25-10%. The treated yarn can be built into yarn packages which can be used in high speed texturizing machines.

Compositions used as spin finishes will preferably have the following compositional range:

|                                                         | Parts by Weight |
|---------------------------------------------------------|-----------------|
| Cycloaliphatic diester                                  | 20-40           |
| High Boiling Aromatic Ester                             | 20-40           |
| Dye Levelling Agent                                     | 10-20           |
| Emulsifiers, depersing agents and/or anti-static agents | 20-30           |

Most preferably, the compositions will contain 25-35 parts by weight of the cycloaliphatic diester and 25-35 parts by weight of high boiling aromatic ester.

Spin finish compositions will preferably contain a cycloaliphatic diester in which R is alkyl of 4-20 carbon atoms, most preferably 6-12 carbon atoms.

The high boiling aromatic ester will preferably be of a glycol, most preferably diesters from ethylene, propylene, or butylene glycol and benzoic or toluic acid.

The dye-levelling agent is preferably an ethoxylated nonylphenol ester, especially of nonylphenol.

The emulsifiers, etc. will preferably comprise ethoxylated castor oil, ethoxylated hydrogenated castor oil and phosphated ethoxylated alkylphenol in ratios of 1:2.2 to 1:3.3 by weight.

A most preferred spin finish composition will consist essentially of:

| Parts by Weight                           |       |
|-------------------------------------------|-------|
| Cycloaliphatic bis(2-ethylhexyl)ester     | 25-35 |
| Propylene glycol dibenzoate               | 25-35 |
| Ethoxylated nonylphenol laurate           | 10-20 |
| Ethoxylated castor oil                    | 4-6   |
| Ethoxylated hydrogenated castor oil       | 8-12  |
| Ethoxylated nonylphenol-phosphate, K salt | 8-12  |

The spin finish compositions can be diluted with water to form a stable emulsion or dispersion for application. The spin finish is preferably applied to produce a pick-up of 0.4-0.75% by weight.

A representative polyester treated to 0.5-0.6% pick-up with the spin finish composition of this invention has lower heat history characteristics than yarn treated with a conventional spin finish. Yarns thus treated can therefore be texturized at lower temperatures than possible heretofore and dyed at lower temperatures than previously used. In addition, the spin finish does not smoke or fume during texturizing at 200°-240° C. In the case of spun yarns, the finish enhances the cohesive properties of the yarn and provides the desired lubricity during picking, cording, drawing, roving and spinning.

It is recommended that, once the spin finishing compositions of this invention have been applied, no conventional lubricants be used, so as to prevent adulteration of the finishes. Maximum benefit is obtained by exclusive use of the compositions of the invention through conversion of the treated yarn to piece goods and dyeing.

#### B. Knitting Application:

The composition is applied to a knitting lubricant and is left on the yarn during subsequent yarn processing. That is, the lubricant need not be scoured off as are conventional lubricants. The capability of omitting a previously required processing step is an important advantage in utilizing the teachings of this invention. During weaving or knitting, high temperatures are reached due to friction and speeds, but the lubricants in accordance with the invention remain functional and do not gum up or build up on equipment. In the dyeing stage, the lubricant/dyeing assistant does not break down during the dyeing cycle (250°-270° F.) and/or smoke during drying and heat setting of the fiber. Elimination of hazy blue smoke during drying and heat setting is important because of increasingly stringent standards against air pollution.

The lubricant compositions of this invention preferably will be of the following composition:

| Parts by Weight             |       |
|-----------------------------|-------|
| Cycloaliphatic diester      | 10-30 |
| High boiling aromatic ester | 30-60 |
| Dye-levelling agent         | 10-30 |
| Emulsifiers, etc.           | 10-30 |

Most preferably, the composition will contain 15-25 parts by weight of cycloaliphatic diester, 35-45 parts by weight of high boiling aromatic ester and 15-25 parts by weight of dye-levelling agent.

The preferred cycloaliphatic diester and dye-levelling agent are as for the spin-finishing composition. However, the high boiling aromatic is preferably a dibenzoate or ditoluate of di- or triethylene glycol or di- or tripropylene glycol.

The conventional emulsifier and anti-static agents preferably are ethoxylated alkylphenols and the corresponding phosphate esters, most preferably ethoxylated nonylphenol.

Other materials in the lubricant composition can include an anti-oxidant, such as butylated hydroxytoluene, in an amount of up to 0.5% by weight; an alkanolamine, such as triethanolamine, in an amount up to 5.0% by weight, and up to 2.5% by weight of water.

A most preferred lubricant composition comprises:

| Parts by Weight                       |          |
|---------------------------------------|----------|
| Cycloaliphatic bis(2-ethylhexyl)ester | 25-35    |
| Dipropylene glycol dibenzoate         | 35-45    |
| Ethoxylated nonylphenol laurate       | 15-25    |
| Ethoxylated nonylphenol               | 5-15     |
| Butylated hydroxytoluene              | 0.05-0.2 |
| Ethoxylated nonylphenol phosphate     | 5-10     |
| Triethanolamine                       | 1-5      |
| Water                                 | 1-2      |

For satisfactory performance, the take up, expressed as minimum percent extractables, when the treated fabric or fiber is loaded into the dyeing machine, should be at least:

| Minimum % extractable       |       |
|-----------------------------|-------|
| Cycloaliphatic diester      | 0.075 |
| High boiling aromatic ester | 0.075 |
| Dye-levelling agent         | 0.050 |

Add-on levels will vary depending on the point in the fiber processing at which the lubricant is applied, but will be from about 0.25 to about 5.0% by weight of the fiber. During knitting, the add-on is preferably 0.5-1.5% by weight.

Another type of knitting lubricant prepared in accordance with the invention will be of the composition:

| Parts by Weight                          |       |
|------------------------------------------|-------|
| Cycloaliphatic diester                   | 5-15  |
| High boiling aromatic ester              | 30-50 |
| Dye-levelling agent                      | 5-15  |
| Emulsifiers, etc.                        | 10-20 |
| Ethylene oxide-propylene oxide copolymer | 10-30 |

The knitting lubricants may also contain up to 0.25% by weight of an anti-oxidant and up to 5% by weight of an alkanolamine, e.g., dibutylethanolamine.

It is preferred that the knitting lubricants contain a cycloaliphatic diester in which R is alkyl of 4-20 carbon atoms, more preferably 6-12 carbon atoms.

The preferred high boiling aromatic ester will be a dibenzoate or ditoluolate of ethylene or propylene glycol. Propylene glycol dibenzoate is particularly preferred.

The dye-levelling agent used in the knitting lubricant composition is preferably an ester of an ethoxylated alkanol, more preferably the decanoate, laurate, myristate or palmitate of ethoxylated decyl, lauryl, myristyl or hexadecyl alcohols.

Ethoxylated alkanols and corresponding phosphates are preferred emulsifiers in the knitting lubricant.

Ethylene oxide-propylene oxide copolymer of molecular weight 2000-5000 is preferred.

A most preferred knitting lubricant is:

| Parts by Weight                          |       |
|------------------------------------------|-------|
| Cycloaliphatic bis(2-ethylhexyl)ester    | 8-12  |
| Propylene glycol dibenzoate              | 35-45 |
| Ethoxylated lauryl laurate               | 8-12  |
| Ethoxylated lauryl alcohol               | 8-12  |
| Butylated hydroxytoluene                 | 0.5-2 |
| Ethylene oxide-propylene oxide copolymer | 20-25 |
| Ethoxylated lauryl alcohol phosphate     | 3-6   |
| Dibutylethanolamine                      | 1-3   |

The lubricant is applied by dripping or misting on to the needles to an uptake of 1-2% on the yarn. The thus-applied composition provides fiber-metal and metal-metal lubrication at temperatures of 100°-150° F. The composition does not break down or gum up the knitting machine.

The foregoing lubricants, if left on the cloth or yarn during the dyeing step, promote uniform dye uptake. In fact, their presence aids dye exhaustion at 240°-270° F. The lubricants do not cause excessive foaming or affect fastness properties of the dyed fabric.

Use of these compositions substantially reduces or eliminates carrier odor and smoke inside and outside processing plants. In addition to reducing air pollution, use of the lubricant compositions of this invention reduces water pollution. Generally, plant surcharges for high BOD/COD or separable oils become unnecessary.

#### C. Application as Coning Oil:

For use as a coning oil, intended for application after texturing or during winding of the yarn, the compositions of this invention will also contain a major amount, up to 70% by weight, of ethylene oxide-propylene oxide copolymers of molecular weight 2000-5000. Exemplary of an appropriate materials are Ucon® LB and HB (Union Carbide Corp.), the Pluronics® (BASF) or Jeffox fluids (Texaco, Inc.).

Coning oil compositions in accordance with the invention will include:

| Parts by Weight                                          |       |
|----------------------------------------------------------|-------|
| Cycloaliphatic diester                                   | 5-10  |
| High boiling aromatic ester                              | 5-10  |
| Dye-levelling agent                                      | 2-5   |
| Emulsifiers, dispersing agents and/or anti-static agents | 10-20 |
| Ethylene oxide-propylene oxide copolymer                 | 60-70 |

Preferred cycloaliphatic diesters for coning oil compositions include those in which R is alkyl of 4-20 carbon atoms, most preferably 6-12 carbon atoms.

The high boiling aromatic ester will preferably be of an alkanol of 8-30 carbon atoms, more preferably decyl, lauryl or myristyl benzoate or toluate.

The dye-levelling agent will preferably be an ester of ethoxylated alkylphenol, more preferably of nonylphenol.

10 The emulsifiers will preferably be ethoxylated alkanols, the corresponding phosphates and ethoxylated hydrogenated castor oil.

Other ingredients in the coning oil compositions can include up to about 0.5% by weight of an antioxidant, such as butylated hydroxytoluene; up to about 2.5% by weight of an alkanolamine, such as triethanolamine and up to 2.5% by weight of water.

A most preferred coning oil formulation is:

| Parts by Weight                          |          |
|------------------------------------------|----------|
| Cycloaliphatic bis(2-ethylhexyl)ester    | 6-8      |
| Lauryl benzoate                          | 6-8      |
| Ethoxylated nonylphenol coconate         | 2-4      |
| Ethoxylated lauryl alcohol               | 8-12     |
| Ethoxylated hydrogenated castor oil      | 2-4      |
| Ethoxylated nonylphenol phosphate        | 2-4      |
| Ethylene oxide-propylene oxide copolymer | 60-70    |
| Butylated hydroxytoluene                 | 0.05-0.2 |
| Triethanolamine                          | 0.5-2    |
| Water                                    | 0.5-2    |

Coning oil in accordance with the invention penetrates the fiber rapidly, but does not sling off the fiber or feeder roll during application. The treated yarn is lubricated sufficiently for the yarn to be rapidly coned, knitted or woven. The composition is stable and does not smoke, yellow or discolor at temperatures up to about 150° F.

#### D. Dyeing:

Dyeing assistant compositions in accordance with the invention will consist of:

| Parts by Weight             |       |
|-----------------------------|-------|
| Cycloaliphatic diester      | 20-40 |
| High boiling aromatic ester | 20-50 |
| Dye-levelling agent         | 10-25 |
| Emulsifiers, etc.           | 10-30 |

The cycloaliphatic diesters utilized for this aspect of the invention will preferably be those wherein R is alkyl of 4-20 carbon atoms, preferably of 6-12 carbon atoms.

Preferred high boiling aromatic esters for this utility are dibenzoates and ditoluolates of mono- and diethylene or propylene glycols.

Dye-levelling agents preferred for this aspect of the invention will be esters of the ethoxylated alkylphenols, particularly ethoxylated nonylphenol.

60 It is preferred that dyeing assistant compositions also contain ethoxylated castor oil and ethoxylated hydrogenated castor oil, as well as the phosphate (potassium salt) of an ethoxylated cycloaliphatic diester, that is, R is phosphated polyoxyethylene.

65 Preferably, the dyeing assistant compositions will contain 25-35 parts by weight of cycloaliphatic diester, 35-45 parts by weight of high boiling aromatic ester and 10-20 parts by weight of dye-levelling agent.

A most preferred dyeing assistant composition will contain:

|                                              | Parts by Weight |
|----------------------------------------------|-----------------|
| Cycloaliphatic bis(2-ethylhexyl)ester        | 25-35           |
| Dipropylene glycol dibenzoate                | 35-45           |
| POE nonylphenol laurate                      | 10-20           |
| POE castor oil                               | 4-6             |
| POE hydrogenated castor oil                  | 8-12            |
| POE cycloaliphatic diester phosphate, K salt | 8-12            |

The composition is applied to the dyebath at a level of 0.25%, based on the weight of the goods. The dye bath is acidic (pH=5±0.5) and contains dye as the only additional ingredient. This is unlike conventional processing requiring a dyeing assistant of 2-4% and other auxiliary levelling agents. Furthermore, the dyeing cycle is less sensitive to rate of temperature change than conventional systems. The dyeing temperature in both systems is usually 265° F. in jet dyeing equipment.

Dyed yarns obtained using the compositions of the invention compare favorably with conventionally dyed yarn in properties such as light-fastness, crocking, shade depth and levelness.

Accordingly, the compositions of this invention, applied to a synthetic fiber when manufactured, or used as a processing aid for texturizing instead of prior art lubricants, both improve the dye affinity of the fiber and generally eliminate the need for further downstream processing and consumption of chemicals associated therewith.

Typical processes or treating agents eliminated include:

- (1) Lubricants during knitting or weaving
- (2) Scour and removal of lubricant
- (3) Dye carrier during dyeing
- (4) Dye dispersant during dyeing
- (5) Dye leveller during dyeing
- (6) Fiber lubricant during dyeing
- (7) Defoamer during dyeing
- (8) Afterclean and scour after dyeing
- (9) Winding lubricant for dyed yarn.

#### DESCRIPTION OF MOST PREFERRED EMBODIMENT

A most preferred general purpose textile-treating composition consists essentially of:

|                                         | Percent by Weight |
|-----------------------------------------|-------------------|
| Bis(2-ethylhexyl)cycloaliphatic ester   | 15-25             |
| Propylene glycol dibenzoate             | 30-50             |
| Polyoxyethylene nonylphenol laurate     | 15-20             |
| Polyoxyethylene hydrogenated castor oil | 5-15              |
| Polyoxyethylene castor oil              | 5-15              |

Without further elaboration, it is believed that one skilled in the art can, using the preceding description, utilize the present invention to its fullest extent. The following specific embodiments are, therefore, to be construed as merely illustrative and not limitative of the remainder of the disclosure in any way whatsoever. In the following examples, the temperatures are set forth uncorrected in degrees Celsius. Unless otherwise indicated, all parts and percentages are by weight.

#### EXAMPLE 1

Preparation of Dialkyl Ester (A is  $-\text{CH}_2\text{CH}_2-$ , R is 2-ethylhexyl).

To three-necked flask fitted with stirrer, thermometer, nitrogen purge, condenser, side-arm receiver and heating mantle were charged 352 g (1 mole) of Diacid 1550, 273 g (2.1 moles) of 2-ethylhexanol, 1.5 g of p-toluenesulfonic acid and 2 g of decolorizing carbon. Air was purged from the flask with nitrogen and the reaction mixture was stirred and heated to 160°-170° C. for 4-6 hours. Water formed during the reaction was collected in the side arm receiver. The reaction was continued until the acid value was below 5 mg KOH/g. The catalyst and carbon were removed by filtration. The ester product and 25 grams of nickel on kieselguhr were charged to a stirred, heated pressure vessel. The mixture was heated to 160°-170° C. and pressurized to 400 psig with hydrogen. A sample was taken after 6-8 hours and the iodine value was determined. The reaction was continued until the iodine value was below 0.5 g of iodine/100 g of sample.

The product was cooled to 50° C. and the catalyst removed by filtration.

Esters are prepared similarly from:

- (1) Diacid 1550 and decyl alcohol, 1:2 molar ratio
- (2) Diacid 1550 and tridecyl alcohol, 1:2 molar ratio
- (3) Diacid 1550 and Neodol 25, a mixture of C<sub>12</sub>-C<sub>15</sub> linear alcohols, 1:2 molar ratio
- (4) Diacid 1550 and butanol, 1:2 molar ratio.

#### EXAMPLE 2

A. Preparation of Polyoxyethylene Diester (A is  $-\text{CH}=\text{CH}-$ , R is HO(CH<sub>2</sub>CH<sub>2</sub>O)<sub>n</sub>CH<sub>2</sub>CH<sub>2</sub>-).

To a stirred autoclave fitted with heating and cooling coils was charged 352 g (1 mole) of Diacid 1550. Catalyst (1.0 g of potassium hydroxide) was charged to the reactor. The temperature was raised to 110° C. and the reactor was vacuum stripped for 30-60 minutes to remove any residual water from previous washing of the reactor or from one or more of the charged reactants or catalyst. The reactor was purged with nitrogen to remove air, evacuated again and purged again with nitrogen. It was stirred and heated to 140° C. and 100 g (2.3 moles) of ethylene oxide was added to the reactor. The pressure inside the reactor immediately built up to 30-50 psig. After 30-60 minutes induction time, an exothermic polymerization reaction (to 150°-160° C.) began with an accompanying pressure drop to zero (0 psig) as ethylene oxide was consumed. Ethylene oxide was added to the reactor to a total of 660 grams (15 moles). The temperature was maintained at 150°-160° C. by cooling. Addition of ethylene oxide was stopped and the reaction was allowed to continue for an additional 30 minutes. The reactor was cooled to 90°-100° C. and purged twice with nitrogen.

A sample of the product had a hydroxyl value of 110 mg of KOH/g (15 moles of ethylene oxide added to the diacid). The diester was acidified with acetic acid to neutralize the potassium hydroxide catalyst and 3 g of hydrogen peroxide was added to bleach and lighten the color of the product. The reactor was cooled to 30° C. and the product was filtered through filter paper using a porcelain filter.

B. Reduction to the Polyoxyethylene Diester (A is  $-\text{CH}_2\text{CH}_2-$ ).

The product of Example 2A and 25 g of nickel on kieselguhr were charged to a stirred, heated pressure

vessel. The mixture was heated to 160°-170° C. and pressurized with hydrogen to 400 psig. After 6-8 hours, samples were removed at intervals for determination of the iodine value. The reaction was continued until the iodine value was less than 0.5 g/100 g of sample.

## EXAMPLE 3

Preparation of Phosphated Polyoxyethylene Diester (A is  $-\text{CH}_2\text{CH}_2-$ , R is



Polyethoxylated (15 moles) diacid, obtained as in Example 2B was heated to 50°-60° C., stirred and purged thoroughly with nitrogen to remove air. To about 1015 g (1.0 mole) of this material was added 24 g (0.17 mole) of  $\text{P}_2\text{O}_5$ . An immediate exothermic reaction occurred (exotherm to 85°-95° C.). The reaction mixture was maintained at this temperature by cooling and an additional 24 g (0.17 mole) of  $\text{P}_2\text{O}_5$  was added. The reaction was continued for 3 hours after all the  $\text{P}_2\text{O}_5$  was added. The reactor was cooled to 50° C. prior to removal of a sample. The product had an acid value of 32 mg KOH/g (indicates the reaction is complete). The batch was bleached at 85°-95° C. with 5 g of hydrogen peroxide, cooled to 30° C. and filtered.

## EXAMPLE 4

Preparation of Propylene Glycol Dibenzoate.

To a 3-necked flask fitted with stirrer, condenser, receiver, thermometer, nitrogen purge and heating mantle were charged 84 g (1.1 mole) of propylene glycol, 244 g (2 moles) of benzoic acid and 0.8 g of p-toluenesulfonic acid. Air was purged from the flask with nitrogen and the contents of the flask were heated to 160°-170° C. Water formed by the reaction was removed continuously. The reaction was continued until the product had an acid value below 5 mg KOH/g. The sample was cooled and filtered.

Other esters are prepared using the following reagents:

- (1) dipropylene glycol and benzoic acid, 1:2 molar ratio
- (2) PPG 200 and benzoic acid, 1:2 molar ratio
- (3) PPG 500 and benzoic acid, 1:2 molar ratio.

## EXAMPLE 5

Preparation of Polyoxyethylene Nonylphenyl Laurate.

To a three-necked flask fitted out as in Example 4 was charged 750 g (1.1 mole) of polyoxyethylated and nonylphenol (9.5 moles of oxyethylene, NP 9.5), 208 g (1 mole) of lauric acid and 2.4 g of p-toluenesulfonic acid. Air was purged from the flask with nitrogen and the mixture was heated to 160°-170° C. until an acid value below 10 mg KOH/g was obtained. The product was cooled and filtered.

Other polyoxyethylene nonylphenyl esters are made in a similar fashion from:

- (1) NP 9.5 and coconut fatty acid, 1:1 molar ratio
- (2) NP 9.5 and oleic acid, 1:1 molar ratio
- (3) NP 9.5 and stearic acid, 1:1 molar ratio
- (4) NP 9.5 and benzoic acid, 1:1 molar ratio.

## EXAMPLE 6

Ethoxylated castor and hydrogenated castor oils were prepared as in Example 2. Ethylene oxide adds to the hydroxyl group of castor oil.

## EXAMPLE 7

A textile-treating composition was made by combining materials prepared as above in the following amounts by weight:

|                                                                      | % by weight |
|----------------------------------------------------------------------|-------------|
| Bis-2-ethylhexyl diester (Example 1)                                 | 20          |
| Propylene glycol dibenzoate                                          | 40          |
| Polyethoxyethylene nonylphenol laurate<br>(9.5 moles ethylene oxide) | 20          |
| Polyethoxyethylene hydrogenated castor<br>(25 moles ethylene oxide)  | 10          |
| Polyethoxyethylene castor<br>(80 moles ethylene oxide)               | 10          |

## EXAMPLE 8

The textile-treating composition of Example 7 was applied during the dyeing cycle to a 10 g swatch of T56 textured polyester test fabric by the following technique:

The sample swatch was placed in a stainless steel beaker containing 150 ml of water, 0.067 g of disperse yellow 67, 0.091 g of disperse red 91, 0.026 g of disperse blue 56, 0.1 g acetic acid (56%) and 0.03 g of the textile-treating composition. The beaker was sealed and placed in a launderometer set at 38° C. The temperature was raised at 4°-5° C. per minute to 130° C. and held for 30 minutes. The beaker was cooled at 4°-5° C. per minute to 52° C. and removed from the launderometer. The polyester swatch was removed from the beaker. It was uniformly dyed in a medium brown shade. Nearly all of the dye was exhausted from the aqueous solution. The swatch was rinsed with cool water and dried in an oven at 121° C.

## EXAMPLE 9

Texturized polyester doubleknit (1500 pounds) were loaded into a 6 port Gaston County jet machine. The machine was filled with water and the goods given an overflow wash. The machine was refilled and ramped to 60° C. Fifteen pounds of acetic acid (56%) and 4.5 pounds of the compositions of Example 7 were dropped into the jet from the drug room. After 5 minutes, 18 pounds of Samaron Yellow 6 GSL (disperse yellow 114), 15 pounds of Bucron Rubine 2BNS (disperse red) and 13 pounds of Foron Blue SBGL (disperse blue 73) were added to the jet machine from the drug room. The jet was sealed off and ramped to 130° C. The temperature was held for 30 minutes at 130° C. and ramped back to 66° C. The fabric was patched for shade, the shade matched standard. The temperature was dropped to 38° C. The spent dye liquor was dropped and the machine refilled with water. The goods were rinsed thoroughly and removed from the jet. The goods were slit, dried and inspected. Final inspection indicated goods of excellent quality.

During the dyeing cycle using the composition of Example 7, the odor level in the dye house was much lower than observed with conventional systems. Little smoking from the ovens was observed during drying

and heat setting at the end of the dyeing cycle. Employee comfort was therefore significantly improved.

The dyeing assistant undergoes facile degradation upon being fed to the plant effluent. The following values were obtained:

|                | Conventional System | Dye Assistant As Above |
|----------------|---------------------|------------------------|
| COD mg/kg      | 2,640,000           | 2,210,000              |
| BOD mg/kg      | <2,000              | 750,000                |
| Ratio, COD:BOD | >1300:1             | 2.95:1                 |

Because little of the dyeing assistant remains on the fabric after dyeing, use of the product of Example 7 does not affect fastness properties of the dyed goods.

The foregoing is typical of production-scale application of the composition.

#### EXAMPLE 10

The procedure of Example 9 was repeated, except that no composition of Example 7 was used. Upon patching at the end of the dyeing cycle, the shade is slightly off due to incomplete dye exhaustion. The bath temperature was taken back up to 132° C. and held an additional 30 minutes. The next patch indicated the shade matched the standard, whereupon the goods were rinsed, removed, slit and dried. Upon inspection, the goods were found to have dye streaks, rope marks, bad barre coverage and a generally unlevel dyeing from end to end and piece to piece. The goods had to be reworked by being loaded back into a dyeing machine and treated with additional dye and levelling agents. The goods were kept in the machine for 3-4 hours until a level dyeing was achieved, but the fabric had a poor appearance as a result of prolonged processing.

This comparative example shows that omission of the composition of the invention produces an unacceptable dyeing.

#### EXAMPLE 11

A textile-treating composition is prepared from the following ingredients:

|                                  | % by weight |
|----------------------------------|-------------|
| bislauryl diester (Example 1)    | 20          |
| dipropylene glycol dibenzoate    | 40          |
| POE (9.5) nonylphenol coconate   | 20          |
| POE (80) castor oil              | 10          |
| POE (25) hydrogenated castor oil | 10          |

This composition is comparable in properties with the composition of Example 7.

#### EXAMPLE 12

A textile-treating composition is prepared as in Example 7, except that 22% by weight of polyoxyethylene diester (Example 2B) and 28% by weight of propylene glycol dibenzoate were used. The composition enhances processing of polyester fabric as described in Example 9.

#### EXAMPLE 13

A textile-processing composition is prepared as in Example 7, except that 18% by weight of phosphated polyoxyethylene diester (Example 3) and 42% by weight of dipropylene glycol dibenzoate are used. The

composition improves the processing of polyester fabric and acts as an anti-static agent.

#### EXAMPLE 14

5 (a) A textile-treating composition was prepared as in Example 7 from the following:

|                                                       | Percent by Weight |
|-------------------------------------------------------|-------------------|
| 10 Cycloaliphatic bis(2-ethylhexyl) ester             | 30.0              |
| Dipropylene glycol dibenzoate                         | 30.0              |
| POE (9.5) nonylphenol laurate                         | 15.0              |
| POE (80) castor oil                                   | 5.0               |
| POE (25) hydrogenated castor oil                      | 10.0              |
| POE (15) diester phosphate potassium salt (Example 3) | 10.0              |

15 (b) The composition thus obtained was applied from a 20% aqueous solution as a spin finish to 150 denier polyester fiber, which was then spun and textured. The finish of the yarn (foy) prior to texturizing was 0.29%; after texturizing foy was 0.25%. The textured yarn built a satisfactory package.

20 25 Spin finish, applied as above, did not smoke, drip, build up on heater plates or cause other undesirable running conditions.

30 The texturized yarn was knitted on an Invoit 18 Gauge machine into a double knit fabric. The yarn knitted well, with a minimum heat build up on the knitting machine. No haze, mist or odor was observed in the knitting plant.

35 The fabric was taken to the dyehouse and loaded into a 6-port Gaston County jet machine. The goods were neither overflow washed nor scoured. Foaming during loading of the fabric was significantly lower than that of fabrics treated with conventional lubricants. The fabric was dyed as in Example 9 to yield a product judged of 40 superior quality. Both dye yield and barre coverage were improved and the fabric had a better overall appearance than untreated fabrics.

#### EXAMPLE 15

45 (a) A spin finishing composition was prepared from:

|                                           | Parts by Weight |
|-------------------------------------------|-----------------|
| 50 Cycloaliphatic bis(2-ethylhexyl) ester | 30              |
| Propylene glycol dibenzoate               | 30              |
| POE (9) nonylphenol laurate               | 15              |
| POE (81) castor oil                       | 5               |
| POE (25) hydrogenated castor oil          | 10              |
| POE (10) nonylphenol phosphate, K salt    | 10              |

55 60 (b) The composition of part (a) was applied, as a 20% emulsion, to polyester yarn (505 denier/34 filament) from a single merge so as to achieve 0.5-0.6% dry pick-up. The treated yarn and yarn treated with a conventional lubricant (Diamond Shamrock FT-504, containing a fatty ester lubricant, nonionic ethoxylate emulsifiers and antistat at 0.5-0.6% pick-up) were textured at 205°-220° C. on a sample Scragg X-2 texturing machine. After texturing, the treated yarns were tested for thermal and other properties. The following results were obtained:

65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8

|                                              | Standard Spin Finish                    | Spin Finish of Example 15(a)            |    |
|----------------------------------------------|-----------------------------------------|-----------------------------------------|----|
| Tube Color                                   | Violet/Green Striped                    | Orange                                  | 5  |
| Denier (short denier method)                 | ~164                                    | ~167                                    |    |
| Filament Count                               | 34                                      | 34                                      |    |
| Density (Density gradient tube method), g/cc | 1.3883<br>(range of 10 samples, 0.0001) | 1.3856<br>(range of 10 samples, 0.0003) |    |
| TMA (Thermomechanical Analysis), °C.         | 165° C.<br>recheck, 168° C.             | 145° C.<br>recheck, 148° C.             |    |
| DSC (Differential Scanning Calorimetry), °C. | 159° C.                                 | 152° C.                                 | 15 |
| % Lubricant (Ether Soxhlet Extraction)       | 0.31                                    | 0.41                                    |    |

TMA is a measure of softening or melting tendency of yarn heated under a constant tension. The decrease in 20 TMA and DSC of the test yarn indicates that the degree of crystallinity is lower than that of yarn treated with a conventional spin finish. Accordingly, treated fibers could be texturized and would absorb dyes at lower temperatures than customary, resulting in decreased 25 energy expenditure.

(c) Photomicrographic studies of yarn cross-sections indicated that both yarns maintained their configurations. Accordingly, it is thought that observed changes in heat history were caused by changes in crystallinity 30 induced by the spin finish applied. Dye penetration of both yarn lots was essentially equivalent, but dye absorption of the fibers treated with the compositions of this Example are higher. The photomicrographs (FIGS. 1-4) also show that the crystallinity of the test specimens has been changed.

(d) Lubricating properties of the yarns was evaluated on the Scragg X-2 machine under varying conditions. The yarn was textured at 340 meters/min at 205°-220° C.

40

The following results were obtained:

| Package No.                                | Disc/Speeds | Yarn Draw Ratio | Center Spindle Tension | Heated Shrinkage |                |      | Break Shrinkage/Elongation |
|--------------------------------------------|-------------|-----------------|------------------------|------------------|----------------|------|----------------------------|
|                                            |             |                 |                        | T <sub>1</sub>   | T <sub>2</sub> | Den. |                            |
| <b>Conventional Spin Finish: (Average)</b> |             |                 |                        |                  |                |      |                            |
| 1                                          | 1.91        | 3.255           | 36.0                   | 44               | 47             | 168  | 15 535/18                  |
| <b>Fiber Finish of Example 15(a):</b>      |             |                 |                        |                  |                |      |                            |
| 1                                          | 1.91        | 3.206           | 36.0                   | 44               | 47             | 170  | 16 515/18.5                |
| 2                                          | 1.91        | 3.255           | 36.0                   | 45               | 50             | 168  | 13 529/18.3                |
| 3                                          | 1.91        | 3.306           | 36.0                   | 47               | 54             | 164  | 13 524/18                  |
| 4                                          | 1.91        | 3.255           | 35.0                   | 51               | 33             | 168  | 14 538/18                  |
| 5                                          | 1.91        | 3.255           | 35.5                   | 47               | 48             | 166  | 15 526/19                  |
| 6                                          | 300 m/m     |                 | 36.0                   | 45               | 49             | 168  | 15 535/18                  |
| 7                                          | 1.91        | 3.255           | 36.5                   | 40               | 65             | 165  | 14 534/17.7                |
| 8                                          | 1.91        | 3.255           | 37.0                   | 38               | 80             | 169  | 12 494/16.6                |
| 9                                          | 1.75        | 3.255           | 36.0                   | 42               | 57             | 166  | 14 501/16.6                |
| 10                                         | 1.96        | 3.255           | 36.0                   | 45               | 47             | 168  | 13 525/17                  |
| 11                                         | 1.99        | 3.255           | 36.0                   | 46               | 46             | 165  | 15 537/17                  |

The frictional properties, breaking strength, elongation and heated shrinkage were judged equivalent.

(e) The effect of texturing temperature on dye uptake of yarn knitted into a sock and dyed was studied from 180°-230° C. Dye absorption by the fiber was measured using a Macbeth Color Eye instrument. The test lot was texturized using the composition of Example 15(a) and contained no other additives. The control lot contained Hipochem TA-3, a commercial dye carrier containing

chlorinated solvents, methylnaphthaline and emulsifiers.

The K/S values (Kubelk-Munk/Scattering) were calculated as follows:

$$K/S = \frac{(1 - \text{reflectance})^2}{2 \times \text{reflectance}}$$

The K/S value is directly proportional to the amount of 10 dye on the fabric.

The following results were obtained:

| Temperature °C. | K/S with Carrier | K/S with Finish of Example 15(a) | % Color Increase |
|-----------------|------------------|----------------------------------|------------------|
| 180             | 5.999            | 6.580                            | 9.7              |
| 185             | 5.907            | 6.510                            | 10.2             |
| 190             | 5.814            | 6.556                            | 12.8             |
| 195             | 5.814            | 6.432                            | 10.6             |
| 200             | 5.721            | 6.426                            | 12.3             |
| 205             | 5.719            | 6.484                            | 13.4             |
| 210             | 5.715            | 6.490                            | 13.6             |
| 215             | 5.816            | 6.542                            | 12.5             |
| 220             | 5.879            | 6.614                            | 12.5             |
| 225             | 5.993            | 6.734                            | 12.4             |
| 230             | 6.151            | 6.888                            | 12.0             |

These results show that the test fabrics had K/S values about 10% higher than a fabric dyed using a conventional carrier. In addition, dye uptake was relatively uniform over a wide temperature range for texturing. These data further indicate that spin finish application is relatively more uniform than heretofore.

(f) Large scale quantities of polyester texturized following use of the spin finish of Example 15(a) were knitted into fabric and dyed in Gaston County Jet Machines without addition of lubricant, leveller, dyeing assistant or dye carrier. The treated polyester consistently gave 7-12% higher color yields than usual. Heat history barre seconds dropped 3-30%, depending on the style and shade.

#### EXAMPLE 16

The lubricant of the following composition was prepared:

|                                       | Parts by Weight |
|---------------------------------------|-----------------|
| Cycloaliphatic bis(2-ethylhexyl)ester | 20.0            |
| Dipropylene glycol dibenzoate         | 39.3            |
| POE (9.5) nonylphenol laurate         | 20.0            |
| POE (10) nonylphenol                  | 10.0            |

-continued

|                                 | Parts by Weight |
|---------------------------------|-----------------|
| Butylated hydroxytoluene        | 0.1             |
| POE (9.5) nonylphenol phosphate | 6.3             |
| Triethanolamine, 98%            | 2.5             |
| Water                           | 1.8             |

## EXAMPLE 17

Coning oil, for application at a level of 2-4% after texturizing, was prepared from:

|                                        | Weight Percent | 15 |
|----------------------------------------|----------------|----|
| cycloaliphatic bis(2-ethylhexyl) ester | 7.50           |    |
| lauryl benzoate                        | 7.50           |    |
| POE (9.5) nonylphenol coconate         | 3.75           |    |
| POE (3.5) lauryl alcohol               | 10.00          | 20 |
| POE (25) hydrogenated castor oil       | 2.50           |    |
| POE (10) nonylphenol phosphate         | 2.50           |    |
| Ucon LB-65                             | 64.15          |    |
| Butylated hydroxytoluene               | 0.10           |    |
| Triethanolamine                        | 1.00           |    |
| Water                                  | 1.00           | 25 |

This coning oil provided necessary lubrication to allow the yarn to be rapidly coned, knitted or woven. It did not smoke, yellow or discolor during processing temperatures of up to 65° C.

## EXAMPLE 18

Knitting lubricant in accordance with the invention was prepared from:

|                                        | Weight Percent |    |
|----------------------------------------|----------------|----|
| Cycloaliphatic bis(2-ethylhexyl) ester | 10.0           | 40 |
| Propylene glycol dibenzoate            | 41.0           |    |
| Lauryl (POE 9) laurate                 | 10.0           |    |
| POE (9) lauryl alcohol                 | 10.0           |    |
| Butylated hydroxytoluene               | 0.1            |    |
| Ucon LB-65                             | 21.9           |    |
| POE (9) lauryl acid phosphate          | 5.0            | 45 |
| Dibutylethanolamine                    | 2.0            |    |

The lubricant was applied to the knitting needles at a level of 1-2% by dripping or misting and was effective as a lubricant at 38°-65° C.

The preceding examples can be repeated with similar success by substituting the generically or specifically described reactants and/or operating conditions of this invention for those used in the preceding examples.

From the foregoing description, one skilled in the art can easily ascertain the essential characteristics of this invention and, without departing from the spirit and scope thereof, can make various changes and modifica-

tions of the invention to adapt it to various usages and conditions.

What is claimed is:

1. A method for lowering heat history characteristics and the degree of crystallinity of a synthetic fiber, lowering the temperature at which the fiber can be texturized and lowering the temperature at which the fiber absorbs dye comprising applying to the fiber to a pick-up of 0.4-0.75% by weight of a composition comprising a cycloaliphatic diester of the formula



wherein R is straight or branched chain alkyl of 4-20 carbon atoms, polyoxyalkylene of the formula  $\text{HO}(\text{CH}_2\text{CH}_2\text{O})_n\text{CH}_2\text{CH}_2-$ ,  $\text{HO}(\text{C}_3\text{H}_6\text{O})_n\text{C}_6\text{H}_3-$ ,  $\text{HO}(\text{CH}_2\text{CH}_2\text{O})_p(\text{CH}_3\text{H}_6\text{O})_q\text{C}_3\text{H}_6-$  or  $\text{HO}(\text{C}_3\text{H}_6\text{O})_p(\text{C}_2\text{H}_4\text{O})_q\text{C}_2\text{H}_4$  or phosphated polyoxyalkylene, wherein n is 2-22 and the sum of p+q is n; and a high boiling aromatic ester of the formula  $\text{ArCOO-R}_1-\text{OOCAr}$  or  $\text{ArCOOR}_2$ , wherein Ar is a substituted or unsubstituted monocyclic aryl of; R<sub>1</sub> is alkylene of 2-8 carbon atoms or polyoxyalkylene of the formula  $-\text{C}_r\text{H}_{2r}(\text{O-C}_s\text{H}_{2s})_s$ , in which r is 2 or 3 and s is up to 15; and R<sub>2</sub> is alkyl or alkenyl of 8-30 carbon atoms; wherein the ratio of cycloaliphatic diester to high boiling aromatic ester is 0.1:1 to 2:1 and wherein the combination of cycloaliphatic diester and high boiling aromatic ester constitutes 10-90% by weight of the composition and texturing the thus-coated fiber at 180°-230° C.

2. The method of claim 1 wherein the composition further comprises a dye-levelling agent of the formula  $\text{R}_3\text{COOR}_4$ , wherein R<sub>4</sub> is an ethoxylated alkylphenol residue of the formula



a is 0-12 and b is 1-24 or an ethoxylated alkanol residue of the formula  $\text{CH}_3(\text{CH}_2)_c-\text{O}-(\text{CH}_2\text{CH}_2\text{O})_d\text{CH}_2\text{C}_\text{H}_2-$ , c is 7-22 and d is 1-24 and wherein R<sub>3</sub> is linear or branched alkyl of 1-21 carbon atoms, phenyl or tolyl.

3. The method of claim 2, wherein the fiber is coated with a minimum extractable of 0.075% by weight of cycloaliphatic diester, 0.075% by weight of high boiling aromatic ester and 0.050% by weight of dye-levelling agent.

4. The method of claim 2, wherein the synthetic fiber is polyester.

5. Polyester fiber treated by the method of claim 1.

\* \* \* \* \*

UNITED STATES PATENT AND TRADEMARK OFFICE  
CERTIFICATE OF CORRECTION

4,293,305

Page 1 of 2

PATENT NO. :

October 6, 1981

DATED

INVENTOR(S) : Robert B. Wilson

It is certified that error appears in the above-identified patent and that said Letters Patent is hereby corrected as shown below:

ABSTRACT, third line after formula: " $\text{HO}(\text{C}_3\text{H}_6\text{O})_n\text{C}_6\text{H}_3-$ ",  
should read --  $\text{HO}(\text{C}_3\text{H}_6\text{O})_n\text{C}_6\text{H}_3-$ , --  
col. 1, line 43: "vol. 57" should read -- vol. 52 --  
col. 6, line 45: "etc. of" should read -- etc. or --  
col. 7, line 51: "applied to" should read -- applied  
as --  
col. 10, line 28: "Butylated hydroxytoluene" should  
read -- Butylated hydroxytoluene --  
col. 12, line 47: "minutes" should read -- minutes' --  
col. 15, line 30: "barre" should read -- barré --  
col. 18, line 1: "methylnaphthaline" should read  
-- methylnaphthalene --  
col. 19, lines 23 and 43: "Butylated hydroxytoluene"  
should read -- Butylated hydroxytoluene --

UNITED STATES PATENT AND TRADEMARK OFFICE  
CERTIFICATE OF CORRECTION

PATENT NO. : 4,293,305

Page 2 of 2

DATED : October 6, 1981

INVENTOR(S) : Robert B. Wilson

It is certified that error appears in the above-identified patent and that said Letters Patent is hereby corrected as shown below:

col. 20, line 20: "HO(C<sub>3</sub>H<sub>6</sub>O)<sub>n</sub>C<sub>6</sub>H<sub>3</sub>-" should read  
-- HO(C<sub>3</sub>H<sub>6</sub>O)<sub>n</sub>C<sub>3</sub>H<sub>6</sub>- --  
col 20, line 21: "HO(CH<sub>2</sub>CH<sub>2</sub>O)<sub>p</sub>(CH<sub>3</sub>H<sub>6</sub>O)<sub>q</sub>C<sub>3</sub>H<sub>6</sub>-" should  
read -- HO(CH<sub>2</sub>CH<sub>2</sub>O)<sub>p</sub>(C<sub>3</sub>H<sub>6</sub>O)<sub>q</sub>C<sub>3</sub>H<sub>6</sub>--  
col. 20, line 49: "aoms" should read -- atoms --.

Signed and Sealed this  
Eighteenth Day of May 1982

[SEAL]

Attest:

Attesting Officer

GERALD J. MOSSINGHOFF

Commissioner of Patents and Trademarks

UNITED STATES PATENT AND TRADEMARK OFFICE  
CERTIFICATE OF CORRECTION

PATENT NO. : 4,293,305

DATED : October 6, 1981

INVENTOR(S) : Robert B. Wilson

It is certified that error appears in the above-identified patent and that said Letters Patent is hereby corrected as shown below:

col. 2, line 39: " $-C_rH_{2r}(O-C_rH_{2r}s)$ " should read  $- -C_rH_{2r}(O-C_rH_{2r}s) - -$

col. 4, line 59: " $-C_rH_{2r}(O-C_rH_{2r}s)$ " should read  $- -C_rH_{2r}(O-C_rH_{2r}s) - -$

Claim 1, line 28: " $-C_rH_{2r}(O-C_rH_{2r}s)$ " should read  $- -C_rH_{2r}(O-C_rH_{2r}s) - -$

Signed and Sealed this

Sixth Day of September 1983

[SEAL]

Attest:

GERALD J. MOSSINGHOFF

Attesting Officer

Commissioner of Patents and Trademarks